



US006875472B2

(12) **United States Patent**  
**Bhattacharya et al.**

(10) **Patent No.:** **US 6,875,472 B2**  
(b5) **Date of Patent:** **Apr. 5, 2005**

(54) **ADHESION PROMOTER APPLICATION SYSTEM AND PROCESS**

(75) Inventors: **Shubho Bhattacharya**, Columbus, OH (US); **Laura McBride**, Powell, OH (US); **Yoshihiro Yamamoto**, West Bloomfield, MI (US); **Shojiro Takeuchi**, FRACC Providencia Jal (MX); **Saul Gonzalez Gutierrez**, Parques Colon Zapopan Jal (MX)

(73) Assignee: **Honda Motor Co., Ltd.**, Tokyo (JP)

(\*) Notice: Subject to any disclaimer, the term of this patent is extended or adjusted under 35 U.S.C. 154(b) by 0 days.

(21) Appl. No.: **10/675,168**

(22) Filed: **Sep. 30, 2003**

(65) **Prior Publication Data**

US 2004/0071886 A1 Apr. 15, 2004

**Related U.S. Application Data**

(63) Continuation of application No. 09/577,776, filed on May 24, 2000, now abandoned.

(51) **Int. Cl.** <sup>7</sup> **B05D 1/36**

(52) **U.S. Cl.** **427/412.3; 427/299; 427/345; 427/372.2; 427/377; 427/378; 427/393.5**

(58) **Field of Search** **427/299, 345, 427/372.2, 377, 378, 393.5, 407.1, 412.3, 421, 424; 118/313, 314, 315, 323**

(56) **References Cited**

**U.S. PATENT DOCUMENTS**

4,214,962 A \* 7/1980 Pincon ..... 204/157.44

4,452,171 A \* 6/1984 Browning ..... 118/58  
4,600,608 A \* 7/1986 Ankrett ..... 427/424  
4,992,216 A \* 2/1991 Saita et al. ..... 261/122.1  
5,230,739 A \* 7/1993 Bartow ..... 118/694  
5,482,745 A \* 1/1996 Cuellar et al. ..... 427/421  
5,534,297 A \* 7/1996 Ogisu et al. ..... 427/322  
5,575,560 A \* 11/1996 Kaneski et al. ..... 366/219  
5,709,947 A \* 1/1998 Hodgkin et al. ..... 428/413  
5,863,333 A \* 1/1999 Kato et al. ..... 118/315  
5,919,288 A \* 7/1999 Mashima et al. ..... 95/155  
6,262,160 B1 \* 7/2001 Kawano et al. ..... 524/378  
6,447,844 B1 \* 9/2002 Kawano et al. ..... 427/302

**FOREIGN PATENT DOCUMENTS**

EP 0 517 471 A2 12/1992  
WO WO 97/31694 A1 \* 9/1997  
WO WO 97/47678 A1 \* 12/1997

\* cited by examiner

*Primary Examiner*—Shrive P. Beck

*Assistant Examiner*—William Phillip Fletcher, III

(74) *Attorney, Agent, or Firm*—Standley Law Group LLP

(57) **ABSTRACT**

A system and method for applying a material for improving the adhesion between the surface of thermoplastic polyolefin (TPO) elements and a coating applied thereto is disclosed. The system comprises the mixing of an adhesion promoter with de-ionized water and applying it to the surface of the TPO elements to be coated. Preferably, the application occurs in an atmospherically controlled enclosure. The application of the adhesion promoter is preferably accomplished by distributing the mixture over the TPO elements through a series of nozzles. Multiple parameters of the application system may be monitored and regulated. Upon completion of the application process, the treated TPO elements are preferably dried in an oven, leaving a thin layer of adhesion promoter over the surface thereof.

**100 Claims, 7 Drawing Sheets**





FIG. 1







FIG. 5



FIG. 6



FIG. 7



FIGURE 8

## 1

ADHESION PROMOTER APPLICATION  
SYSTEM AND PROCESSCROSS-REFERENCE TO RELATED  
APPLICATIONS

This application is a continuation of application Ser. No. 09/577,776, filed May 24, 2000 now abandoned, for Adhesion Promoter Application System and Process, which is expressly incorporated herein by reference.

BACKGROUND AND SUMMARY OF THE  
INVENTION

Environmental concerns have led to an attempted reduction of pollutants from a multitude of sources. Manufacturing facilities, have been required to operate under increasingly stringent emissions guidelines. These emissions guidelines require, in part, a reduction of volatile organic compound (VOC) emissions.

In a manufacturing environment, VOC's have a wide variety of uses. For example, certain VOC's have been commonly employed for the purpose of cleaning and preparing various plastic components for receiving a material coating, such as paint. More specifically, such VOC's are particularly useful for cleaning and preparing thermoplastic polyolefin (TPO) components for coating with a primer or paint product. Not only are such VOC's effective for the removal of grease and other contaminants which may reside on these components, they also act on the surface of the TPO to promote adhesion with the forthcoming primer or paint coating.

In an attempt to reduce emissions, it has become essential to drastically reduce or eliminate the use of VOC's. For similar reasons, most automobile manufacturers also now employ a water-based paint and/or primer rather than traditional solvent-based products.

New plastic formulations have been developed which may be cleaned via non-VOC methods, and which are better able to bond with water-based paint and/or primer. However, TPO exhibits inherently poor wettability—meaning that it tends to repel moisture. Without the use of trichloroethylene or similar materials to prepare the surface, providing adequate paint adhesion is of great concern. For this reason, manufacturers utilizing a water-based cleaning system and water-based paint, typically provide the TPO components with a primer coat prior to the final paint or color coat.

Unfortunately, primer coating is a costly process. One reason is that a large portion of the sprayed primer is typically lost rather than deposited on the component. Additionally, once the components have received a primer coat, it is generally necessary to cycle them through an oven to allow the primer to fully dry. Therefore, it is desirous to develop a system and method that will allow a paint coating to be applied directly to the surface of a TPO component, without the need to first apply a coat of primer.

The present invention satisfies this need. The system and method of the present invention applies a water-based adhesion promoter to each TPO component. The adhesion promoter application preferably occurs after the component has undergone a cleaning process. After the adhesion promoter is applied and dried, a thin layer will remain on the surface of the TPO component. This thin layer of adhesion promoter is sufficient to provide the necessary adhesion between the component and the forthcoming paint coat.

The adhesion promoter application system of the present invention may monitor a variety of parameters during

## 2

operation, including, for example: line speed of the component; temperature of the component; temperature of the adhesion promoter; adhesion promoter nozzle distance and angle; adhesion promoter flow rate; nozzle spray pattern; setting zone time, temperature and relative humidity; and pre-oven and oven time, temperature and relative humidity. The adhesion promoter application system of the present invention may also be adapted to distinguish when a part is present within the system and to provide periodic water flushing in order to prevent adhesion promoter build-up.

Therefore, the adhesion promoter application system of the present invention allows a paint coat to be applied to the surface of a TPO component without the need to first apply a primer coat. As such, the present invention may provide a reduction in material, equipment and labor costs, as well as an increase in production capacity.

## BRIEF DESCRIPTION OF THE DRAWINGS

In addition to the novel features and advantages mentioned above, other objects and advantages of the present invention will be readily apparent from the following descriptions of the drawings and embodiments, wherein:

FIG. 1 is a schematic diagram illustrating various components comprising one embodiment of the system of the present invention;

FIG. 2 is a pictorial diagram depicting a typical prior art TPO component coating system;

FIG. 3 is a pictorial diagram depicting an embodiment of the TPO component coating process disclosed by the present invention;

FIG. 4 graphically illustrates the stages of one embodiment of the adhesion promoter application process of the present invention;

FIG. 5 is an enlarged front view, showing a series of TPO components passing through an application portion of one embodiment of the adhesion promoter application system of the present invention;

FIG. 6 is an enlarged side view, in partial cross-section, depicting several components of the application portion of the embodiment of the adhesion promoter application system shown in FIG. 5;

FIG. 7 illustrates alternate embodiments of adhesion promoter application nozzles utilized in the present invention; and

FIG. 8 is a schematic diagram detailing the operating procedure of a particular embodiment of the present invention.

DETAILED DESCRIPTION OF THE  
EMBODIMENT(S)

A schematic representation of various components of one embodiment of the adhesion promoter application system 10 of the present invention can be seen in FIG. 1. A treatment enclosure 15, which may be a portion of a larger pretreatment enclosure, provides a captive environment for the application of the adhesion promoter to particular thermoplastic polyolefin (TPO) elements (not shown).

The treatment enclosure 15 is preferably closed at its entrance by a first air seal 20, and at its exit by a second air seal 25. A fan 30 may provide the air supply necessary to maintain the air seals 20, 25. The TPO elements are preferably cooled prior to entering the treatment enclosure 15, thus, the first air seal 20 helps to prevent cool air from entering the treatment enclosure. A pre-oven is preferably

connected to the exit portion of the treatment enclosure 15. Similar in function to the first air seal 20, the second air seal 25 helps to prevent hot air from the pre-oven from entering the treatment enclosure 15. An air temperature and humidity conditioner 35 is preferably provided to maintain the atmospheric conditions within the treatment enclosure 15. A chiller 40 and a boiler 45 are provided to supply cooled and heated water, respectively, to the air temperature and humidity conditioner 35.

A supply tank 50 is preferably utilized to maintain a source of an adhesion promoter for use by the system 10. A stock of adhesion promoter 55 and a supply of de-ionized water 60 are preferably in metered communication with the supply tank 50. The adhesion promoter stock 55 is further metered and controlled by a surface tension meter 65. The surface tension meter 65 is adapted to analyze a wet sample of adhesion promoter, and thereby control the amount of adhesion promoter and solvent that is supplied to the supply tank 50. A re-circulation pump 70 is preferably used to re-circulate the adhesion promoter through an ultra-filtration module 75 for removing particulate contamination.

The adhesion promoter in the supply tank 50 is preferably supplied to a gravity tank 80 by means of a supply pump 85. The adhesion promoter preferably passes through a supply filter 90, and also passes through a heat exchanger 95 on its way to the gravity tank 80. The heat exchanger 95 operates to adjust the temperature of the adhesion promoter traveling to the gravity tank 80. Preferably, the temperature of the adhesion promoter in the gravity tank is maintained at between about 20–25° C. The chiller 40 and boiler 45 also supply cooled and heated water, respectively, to the heat exchanger 95.

From the gravity tank 80, the adhesion promoter is preferably directed to a multitude of nozzles 100 within the treatment enclosure 15 for application to the passing TPO elements. The temperature of the adhesion promoter may be monitored within the gravity tank 80 and the flow rate may be monitored at the nozzle 100 outlets to ensure proper application to the TPO elements. Operation and monitoring of the system 10 may be conducted via an operator/electrical panel 105.

Alternate embodiments may also be possible. For example, the stock of adhesion promoter 55 and supply of de-ionized water 60 may be supplied directly to the gravity tank 80 or directly to the nozzles 100. Alternatively, the supply tank 50 may be used without the gravity tank 80, whereby the adhesion promoter may be supplied directly from the supply tank to the nozzles 100.

FIG. 2 illustrates a known TPO element coating process 120. TPO elements traveling in a direction indicated by the arrows first enter a pretreatment enclosure 125. Within the pretreatment enclosure 125, the elements are subjected to a washing/degreasing process, and typically, to a surface conditioning operation. Upon exiting the pretreatment enclosure 125, the TPO elements enter a primer booth 130, where a coat of primer is applied to promote adhesion between the TPO element and a later applied base coat. The primed TPO elements are then passed through a primer oven 135 in order to fully dry the primer coat. After the primer coat is fully dried in the primer oven 135, the TPO elements enter a paint booth 140, where they receive a base (color) coat and possibly a clear coat. The base coat, and if applicable the clear coat, are then dried in a paint oven 145 prior to their availability for final use.

An overview of the TPO element coating process 150 of the present invention can be seen by reference to FIG. 3. In

the present invention the TPO elements, traveling in the direction of the arrows, enter a pretreatment enclosure 155. Within the pretreatment enclosure 155, the TPO elements preferably undergo a washing/degreasing process and are then subjected to application of the adhesion promoter in a treatment section of the enclosure. Because the adhesion promoter allows a base coat to be applied directly to the adhesion promoter-treated surface of the TPO elements, the need for a primer booth and primer oven is obviated. Therefore, as shown in FIG. 3, upon exiting the pretreatment enclosure 155, the TPO elements may enter directly into a paint booth 160, where they receive a base (color) coat and possibly a clear coat. The base coat, and if applicable the clear coat, are then dried in a paint oven 165 prior to their availability for final use.

Another advantage to the process of the present invention is depicted in FIG. 3. Because no primer booth or primer oven is required, at least one additional paint booth 170 and paint oven 175 may be available for receiving adhesion promoter-treated parts. The additional paint booth 170 and paint oven 175 may be created by converting a pre-existing primer booth and primer oven, for example. Thus, the adhesion promoter application system and process of the present invention may also serve to double the production capacity of the TPO element paint process.

A graphical representation of the various stages of an embodiment of the adhesion promoter application process 200 of the present invention can be seen in FIG. 4. For purposes of clarity, the enclosure portion of the system is represented as transparent. It should also be noted that although a carrier 225 is shown in FIG. 4 to hold only one TPO element 210, it is possible, and typically desirable that each carrier transport multiple elements.

The TPO element 210, represented in this embodiment as an automobile bumper fascia, can be seen near a cooling portion 215 of a pretreatment enclosure 220. As represented in this position, the TPO element 210 has already been subjected to a washing/degreasing operation in a more forward portion (not shown) of the pretreatment enclosure 220.

Because the temperature of the TPO element 210 has likely become elevated during the washing/degreasing operation, the TPO element is transported in the direction of the arrows by the carrier 225, and through a cooling device 230. For purposes of illustration, the cooling device 230 may be a series of nozzles spraying cooled, de-ionized water, as represented here, but other embodiments are also possible that can produce the desired effect. The cooling device 230 preferably reduces the temperature of the TPO element 210 to approximately that of the adhesion promoter application section 235 of the pretreatment enclosure 220. Cooling of the TPO element 210 is desirable to prevent heat transfer from the TPO element to the atmosphere within the adhesion promoter application section 235 of the pretreatment enclosure 220.

A first air seal 240, preferably created by a fan 30 (FIG. 1), assists in preventing the atmosphere of the cooling portion 215 of the pretreatment enclosure 220 from influencing the atmosphere within the adhesion promoter application section 235. The temperature of the first air seal 240 is preferably maintained at approximately the desired interior temperature of the adhesion promoter application section 235 of the pretreatment enclosure 220.

The TPO element 210 and carrier 225 pass through the first air seal 240 and into the adhesion promoter application section 235 of the pretreatment enclosure 220. A second air

seal 245 separates the adhesion promoter application section 235 of the pretreatment enclosure 220 from a pre-oven 265. At a point preferably nearer the first air seal 240, an application portion 250 (FIGS. 5-7) of the adhesion promoter application system applies the adhesion promoter 255 to the TPO element 210. The linear velocity of the carrier 225 and TPO element 210 during application of the adhesion promoter is preferably between approximately 1-5 meters per minute, and in one example embodiment, is approximately 1.2 meters per minute.

The remaining segment of the adhesion promoter application section 235 of the pretreatment enclosure 220 located between the application portion 250 and the second air seal 245 is used as a setting zone 260. The setting zone 260 allows at least a portion of the adhesion promoter to flash off of the TPO element 210 before entering the pre-oven 265. Preferably, the adhesion promoter application section 235 of the pretreatment enclosure 220 is maintained at a temperature of between about 20-25° C. and a relative humidity of between approximately 40-70%.

Upon exiting the adhesion promoter application section 235 of the pretreatment enclosure 220 through the second air seal 245, the TPO element 210 preferably enters a pre-oven 265, where the temperature of the TPO element and the remaining adhesion promoter is elevated prior to entering a drying oven 270. The temperature may vary from between approximately 25-65° C., and the relative humidity may vary from between about 15-60% depending on the location of the TPO element 210 within the pre-oven 265.

The adhesion promoter remaining on the TPO element 210 is preferably further dried in the drying oven 270 prior to entering a paint booth 160, 170 (FIG. 3). The temperature may vary from between approximately 45-95° C., and the relative humidity may vary from between about 5-25% depending on the location of the TPO element 210 within the drying oven 270.

An enlarged, frontal view of an embodiment of the application portion 300 of the adhesion promoter application system is shown in FIG. 5. Multiple TPO elements 210 can be seen to be placed in communication with a supply of an emitted adhesion promoter 310 by the carrier 225. In this embodiment, the adhesion promoter 310 is supplied, preferably via a gravity tank (not shown), to a main and secondary supply header 315, 320. The use of a gravity tank helps to prevent foaming of the adhesion promoter 310 as it contacts the TPO elements 210, by reducing the amount of air trapped therein. It has been found that excessive foaming may lead to defects, such as streaks, runs, and sags in the layer of adhesion promoter deposited on the TPO elements 210.

Each of the main and secondary supply headers 315, 320 are shown to have multiple nozzles 325, 330 for distributing the adhesion promoter 310 upon the TPO elements 210 passing underneath. Although the number of nozzles 325, 330 may vary, good results have been achieved by using between about 15-30 total nozzles.

The nozzles may be of differing configuration to allow for various adhesion promoter 310 distribution patterns. Various shapes, such as a stream 335 or a fan pattern 340, for example, may be employed to most appropriately distribute the adhesion promoter 310 about the TPO components 210 without causing defects.

Each of the nozzles 325, 330 preferably also possesses its own flow control device (not shown). The flow control device may be a manual valve, or an electronic solenoid operated valve, for example. The use of a flow control

device is preferred, as it has been found that the flow rate of the adhesion promoter 310 can affect the quality of the final adhesion promoter layer that will remain on each of the TPO components 210. Satisfactory results have been achieved using an adhesion promoter flow rate of between approximately 0.5-2.5 liters per minute, and in one example embodiment, the adhesion promoter flow rate is approximately 1.5 liters per minute.

FIG. 6 is an enlarged side view, in partial cross-section, which illustrates the supply headers 315, 320 and nozzles 325, 330 of FIG. 5 in more detail. A cross-section of typical header 315, 320 construction is shown to be partially filled with the adhesion promoter 310. The headers 315, 320 may be manufactured of various materials, such as, for example, PVC pipe. The nozzles 325, 330 extend from the headers 315, 320 and are in communication with the adhesion promoter 310 located therein. The nozzles 325, 330 may be constructed of various types and sizes of pipe or tubing, and are preferably manufactured of a plastic or stainless steel material. As discussed above, it is also preferable that the nozzles 325, 330 possess some type of flow control (not shown).

As can be seen, the nozzles 325, 330 are preferably angled in the direction of travel of the TPO elements 210, which direction is indicated by the arrow. Delivering the adhesion promoter 310 through an angled nozzle 325, 330 appears to reduce the force of impact on the TPO element 210 by the adhesion promoter, thereby reducing foaming and subsequent adhesion promoter layer defects. Although the optimum angle  $\phi$  of the nozzles may vary depending on the configuration of the TPO element 210 to which the adhesion promoter 310 is to be applied, good results have been obtained utilizing a nozzle angle  $\phi$  of between about 10-45 degrees relative to vertical. However, based upon factors such as TPO element configuration, TPO element linear velocity, adhesion promoter flow rate, and nozzle to element distance, for example, lesser or greater nozzle angles may also give satisfactory results.

As also shown in FIG. 6, it may be preferable to position the TPO element 210 at an angle  $\beta$  as it passes beneath the adhesion promoter 310. In the embodiment of FIG. 6, the TPO element 210 is shown to be angled on the carrier 225, toward its direction of travel and away from the nozzles 325, 330. It has been found that orienting the TPO element 210 as shown may reduce the amount or severity of defects appearing in the adhesion promoter layer that remains on the TPO element after drying. As with the nozzle angle  $\phi$  discussed above, the optimum angle  $\beta$  of TPO element 210 orientation on the carrier 225 will depend largely on the configuration of the TPO element and other application parameters. However, good results have been achieved for the embodiment illustrated in FIG. 6 by orienting the TPO element 210 on the carrier 225 at an angle  $\beta$  of between about 5-20 degrees, and more preferably about 12 degrees from vertical, in a direction away from the nozzles 325, 330.

Now referring to FIG. 7, a frontal, detailed view of the nozzles 325, 330 of FIGS. 5 and 6 can be seen. Three different types of nozzles 325, 330 are shown to extend from the supply header 315, 320. A single stream nozzle 350 is shown on the right. The single stream nozzle 350 is adapted to deliver an adhesion promoter stream 355 of substantially uniform diameter to the TPO element 210. A dispersion nozzle 360 is seen in the middle position. The dispersion nozzle 360 is designed to apply a wider pattern 365 of the adhesion promoter to the TPO element 210. A fan nozzle 370 can be seen on the left. The fan nozzle 370 preferably has a thin opening 380 of between approximately 20-30

millimeters in width, which causes the adhesion promoter **310** to exit the nozzle in substantially a fan pattern **375**. Depending on the distance between the nozzles **325**, **330** and the TPO element **210**, the length L of the fan portion **375** of the adhesion promoter stream **385** is preferably between about 10–150 millimeters.

A variety of nozzle diameters **390** may be employed to adequately expel the adhesion promoter **310**. However, for the embodiments illustrated in FIGS. 5–7, the best results have been achieved by using a nozzle diameter of between approximately 0.25–0.50 inches, with a nozzle opening diameter **395** of between about 0.5–1.0 millimeters.

It has been discovered through experimentation that the distance D between the nozzles **325**, **330** and the surface of the TPO element **210** also may have bearing on the quality of the adhesion promoter layer that will be deposited thereon. As with flow rate and angle of impact, it appears that the distance D between the nozzles **325**, **330** and the surface of the TPO element **210** affects the amount of splashing and foaming of the adhesion promoter **310** that will occur. Depending on adhesion promoter flow rate, linear speed of the TPO elements **210**, and TPO element configuration, a distance D of between approximately 0.25–14 inches has yielded acceptable results. For the embodiments shown in FIGS. 5–7, however, a distance D of approximately 1.75 inches is preferable. Due to variations in distance D that may be required between different TPO elements, it is preferable that a part collision detection limit switch means be employed to ensure that a TPO element is not able to collide with any of the nozzles **325**, **330**.

The operating procedure of a particular embodiment of the present invention can be seen in the diagram of FIG. 8. A master on switch **410**, which delivers electrical power to the system, is first activated. Electrical power is then in turn applied, either by manual activation or automatically, to: the TPO element conveyor **415**, which is constrained via an interlock to check the condition of one or more part collision detection limit switches **420**; the air seal fan **425**; and the air conditioning (atmosphere control) fan **430**. Upon activation of the air conditioning fan **430**, a signal is sent from both an enclosure temperature sensor **435** and an enclosure humidity sensor **440**. The enclosure temperature sensor **435** and enclosure humidity sensor **440** are in respective communication with a modulating valve for the hot water return from the air-conditioning coil **445** and a modulating valve for the chilled water return from the air-conditioning coil **450**. This allows for automatic control of the temperature and relative humidity within the enclosure **15**. A check is then made to verify that both the chiller and boiler are operational **455**.

Next, electrical power is applied to a pump for supplying the adhesion promoter **460**. Upon activation of the adhesion promoter pump **460**, an adhesion promoter tank temperature sensor **465**, which is in communication with both a modulating valve for the hot water return from the heat exchanger **470** and a modulating valve for the chilled water return from the heat exchanger **475**, operates to maintain the desired temperature of the adhesion promoter. Activation of the adhesion promoter pump **460** also triggers a check of adhesion promoter on/off flow control valves **480**, and part-gap detection photo sensors **485**, which evaluate the position of the adhesion promoter application nozzles in relation to the TPO elements to be treated. The adhesion promoter on/off flow control valves **480** are also interconnected to a solenoid valve for de-ionized water nozzle purging **490**, which periodically provides de-ionized water to the nozzles to prevent the build-up of adhesion promoter.

A filtration pump **495** and a de-ionized water pump **500** are then turned on. The energizing of the de-ionized water

pump **500** activates a de-ionized water temperature sensor **505**. The de-ionized water temperature sensor **505** is in communication with the modulating valve for the chilled water return from the heat exchanger **510**, which allows the temperature sensor **505** to control the temperature of the de-ionized water supply that may be used, among other things, to rinse and cool the TPO elements prior to application of the adhesion promoter.

An adhesion promoter tank pH sensor is next activated **515**, along with an adhesion promoter tank electrical conductivity sensor **520**. The pH sensor **515** and the conductivity sensor **520** allow the properties of the adhesion promoter to be monitored.

The scope of the invention is not to be considered limited by the above disclosure, and modifications are possible without departing from the spirit of the invention as evidenced by the following claims:

What is claimed is:

1. A method of improving adhesion between the surface of one or more thermoplastic polyolefin elements and a paint coat subsequently applied thereto, said method comprising:
  - 20 supplying an adhesion promoter;
  - creating a mixture of said adhesion promoter and de-ionized water;
  - providing an enclosure, said enclosure forming a protective environment for the application of said mixture;
  - 25 regulating the atmosphere within said enclosure;
  - providing said mixture to an application device located within said enclosure said application device having at least one nozzle;
  - 30 placing said one or more thermoplastic polyolefin elements within said enclosure;
  - 35 applying said mixture to said one or more thermoplastic polyolefin elements via said at least one nozzle of said adhesion promoter application device, such that said mixture flows over said one or more thermoplastic polyolefin elements;
  - 40 regulating at least the angle and velocity at which said mixture contacts said one or more thermoplastic polyolefin elements; and
  - 45 drying said one or more thermoplastic polyolefin elements after application of said mixture;
  - 50 whereby a dried layer of said adhesion promoter is retained on the surface of said one or more thermoplastic polyolefin elements; and
  - 55 wherein application of said mixture according to said method minimizes agitation of said mixture and thereby reduces or eliminates defects in said dried layer of adhesion promoter.
2. The method of claim 1, wherein the average flow rate of said mixture through said at least one nozzle is between about 0.5–2.5 liters per minute.
3. The method of claim 1, wherein the distance between said at least one nozzle and the surface of said thermoplastic polyolefin elements is between about 0.25–14 inches.
4. The method of claim 1, wherein said adhesion promoter application device has between about 15–30 total nozzles.
5. The method of claim 1, wherein the diameter of said at least one nozzle is between approximately 0.25–0.5 inches.
6. The method of claim 1, wherein the opening diameter of said at least one nozzle is between approximately 0.5–1.0 millimeters.
7. The method of claim 1, wherein said at least one nozzle is oriented at an angle of between 10–45 degrees relative to vertical.

8. The method of claim 7, wherein said orientation of said at least one nozzle is toward the direction of travel when said thermoplastic polyolefin elements travel through said application of said mixture.

9. The method of claim 1, further comprising moving said thermoplastic polyolefin elements through the application of said mixture by said adhesion promoter application device.

10. The method of claim 9, wherein the linear velocity of said thermoplastic polyolefin elements is between about 1–5 meters per minute.

11. The method of claim 9, wherein said thermoplastic polyolefin elements are oriented at an angle away from the direction of application of said mixture when said mixture is applied at an angle.

12. The method of claim 11, wherein said angle is between about 5–20 degrees.

13. The method of claim 1, further comprising cleaning said thermoplastic polyolefin elements prior to said application of said mixture.

14. The method of claim 13, further comprising rinsing said thermoplastic polyolefin elements with de-ionized water prior to application of said mixture.

15. The method of claim 1, further comprising adjusting the temperature of said thermoplastic polyolefin elements to approximately the temperature of the portion of said enclosure that houses said adhesion promoter application device.

16. The method of claim 15 wherein said temperature is between about 20–25° C.

17. The method of claim 1, further comprising maintaining the relative humidity within said enclosure at between approximately 40–70%.

18. The method of claim 1, wherein the amount of said adhesion promoter mixed with said water is regulated by a metering device.

19. The method of claim 18 wherein a surface tension meter is adapted to analyze a wet sample of said mixture, said surface tension meter communicating with said metering device to provide regulation of the amount of said adhesion promoter added to said water based on said analysis.

20. The method of claim 1, further comprising providing a storage device for receiving an amount of said mixture.

21. The method of claim 20, further comprising re-circulating said mixture within said storage device.

22. The method of claim 21, further comprising filtering said mixture during said re-circulation.

23. The method of claim 1, further comprising passing said mixture through a heat exchanger to regulate the temperature of said mixture prior to application by said adhesion promoter application device.

24. The method of claim 23, wherein said means for supplying said mixture to said application device supplies said mixture from said heat exchanger to said adhesion promoter application device.

25. The method of claim 24, wherein said means for supplying said mixture to said application device supplies said mixture from said heat exchanger to a gravity tank.

26. The method of claim 25, wherein said gravity tank supplies said mixture to a supply header located within said enclosure.

27. The method of claim 26, wherein said supply header has at least one nozzle extending therefrom and in communication with said mixture located therein, said supply header and said at least one nozzle forming at least a portion of said adhesion promoter application device.

28. The method of claim 1, further comprising the use of at least a partial seal for sealing each end of said enclosure.

29. The method of claim 28, wherein said at least a partial seal is an air seal.

30. The method of claim 29, wherein said air seal is provided by a fan.

31. The method of claim 1, wherein said drying of said thermoplastic polyolefin elements occurs in an oven.

32. The method of claim 31, wherein the temperature within said oven is between about 45–95° C.

33. The method of claim 31, wherein the relative humidity within said oven is between about 5–25%.

34. The method of claim 31, wherein said thermoplastic polyolefin elements enter a pre-oven prior to entering said oven.

35. The method of claim 34, wherein the temperature within said pre-oven is between about 25–65° C.

36. The method of claim 34, wherein the relative humidity within said pre-oven is between about 15–60%.

37. A method of improving adhesion between the surface of a thermoplastic polyolefin element and a subsequently applied paint coat, said method comprising:

supplying a mixture of an adhesion promoter and de-ionized water;

providing an application enclosure, said enclosure forming a protective environment for the application of said mixture;

regulating the atmosphere within said application enclosure;

providing said mixture to a plurality of nozzles located within said application enclosure;

locating said thermoplastic polyolefin element within said application enclosure;

applying said mixture to said thermoplastic polyolefin element using said plurality of nozzles, such that said mixture flows over said thermoplastic polyolefin element;

regulating, during application of said mixture to said thermoplastic polyolefin element, one or more of a flow rate of said mixture, a discharge pattern of said plurality of nozzles, an angle of said plurality of said nozzles, a distance of said plurality of nozzles from said thermoplastic polyolefin element, and an orientation of said thermoplastic polyolefin element, in order to cover said thermoplastic polyolefin element with said mixture while minimizing the agitation thereof; and

drying said thermoplastic polyolefin element in a drying enclosure after application of said mixture;

whereby a dried layer of said adhesion promoter is retained on the surface of said thermoplastic polyolefin element; and

wherein application of said mixture to said thermoplastic polyolefin element in such a manner minimizes or eliminates defects in said dried layer of adhesion promoter.

38. The method of claim 37, wherein the average flow rate of said mixture through said plurality of nozzles is between about 0.5–2.5 liters per minute.

39. The method of claim 37, wherein the distance between said plurality of nozzles and the surface of said thermoplastic polyolefin element is between about 0.25–14 inches.

40. The method of claim 37, wherein there are between about 15–30 total nozzles.

41. The method of claim 37, wherein the diameter of said plurality of nozzles is between approximately 0.25–0.5 inches.

42. The method of claim 37, wherein the opening diameter of said plurality of nozzles is between approximately 0.5–1.0 millimeters.

## 11

43. The method of claim 37, wherein at least some of said plurality of nozzles are oriented at an angle of between about 10–45 degrees relative to vertical.

44. The method of claim 43, further comprising moving said thermoplastic polyolefin element through said application of said mixture by said plurality of nozzles.

45. The method of claim 44, wherein said angle of said at least some of said plurality of nozzles is toward a direction of travel of said thermoplastic polyolefin element.

46. The method of claim 44, wherein the linear velocity of said thermoplastic polyolefin element is between about 1–5 meters per minute.

47. The method of claim 44, wherein said thermoplastic polyolefin element is angled toward a direction of travel of said thermoplastic polyolefin element.

48. The method of claim 47, wherein said angle is between about 5–20 degrees.

49. The method of claim 37, further comprising cleaning said thermoplastic polyolefin element prior to said application of said mixture.

50. The method of claim 49, further comprising rinsing said thermoplastic polyolefin element with de-ionized water prior to application of said mixture.

51. The method of claim 37, further comprising adjusting the temperature of said thermoplastic polyolefin element to approximately the temperature within said application enclosure.

52. The method of claim 51, wherein said temperature is between about 20–25° C.

53. The method of claim 37, wherein said atmosphere within said application enclosure is maintained at between approximately 40–70% relative humidity.

54. The method of claim 37, wherein the amount of adhesion promoter mixed with water is regulated by a metering device.

55. The method of claim 54, wherein a surface tension meter is adapted to analyze a wet sample of said mixture, said surface tension meter communicating with said metering device to provide regulation of the amount of said adhesion promoter added to said water based on said analysis.

56. The method of claim 54, wherein said water is de-ionized water.

57. The method of claim 37, further comprising providing a storage device for receiving and storing an amount of said mixture.

58. The method of claim 57, further comprising re-circulating said mixture within said storage device.

59. The method of claim 58, further comprising filtering said mixture during re-circulation.

60. The method of claim 37, further comprising passing said mixture through a heat exchanger to regulate the temperature of said mixture prior to application by said plurality of nozzles.

61. The method of claim 60, wherein a pump supplies said mixture from said heat exchanger to said plurality of nozzles.

62. The method of claim 60, wherein a pump supplies said mixture from said heat exchanger to a gravity tank.

63. The method of claim 62, wherein said gravity tank supplies said mixture to a supply header located within said enclosure.

64. The method of claim 63, wherein said plurality of nozzles are in communication with said mixture located in said supply header.

65. The method of claim 37, further comprising the use of at least a partial seal for sealing each end of said enclosure.

## 12

66. The method of claim 65, wherein said seal is an air seal.

67. The method of claim 66, wherein said air seal is provided by a fan.

68. The method of claim 37, wherein the temperature within said drying enclosure is between about 45–95° C.

69. The method of claim 37, wherein the relative humidity within said separate drying enclosure is between about 5–25%.

70. The method of claim 37, wherein said thermoplastic polyolefin element enters a pre-oven prior to entering said drying enclosure.

71. The method of claim 70, wherein the temperature within said pre-oven is between about 25–65° C.

72. The method of claim 70, wherein the relative humidity within said pre-oven is between about 15–60%.

73. A method of improving adhesion between a thermoplastic polyolefin element and a subsequently applied paint coat by depositing a layer of an adhesion promoter on the surface of said element, said method comprising:

supplying an adhesion promoter;

forming an adhesion promoter mixture from said adhesion promoter and de-ionized water;

providing a mixture storage tank for receiving and storing a supply of said mixture;

transferring at least a portion of said mixture to said mixture storage tank;

providing a mixture application enclosure, said mixture application enclosure having a regulated atmosphere and forming a protective environment around said thermoplastic polyolefin element during application of said mixture thereto;

providing a gravity tank for receiving a supply of said mixture from said mixture storage tank;

providing at least one supply header for receiving, via gravity from said gravity tank, an amount of said mixture;

providing a plurality of nozzles in communication with said at least one supply header said plurality of nozzles adapted to be adjustable in location and direction, and to distribute said mixture received from said gravity tank over the surface of said thermoplastic polyolefin element;

locating said thermoplastic element on a carrier;

cooling said thermoplastic polyolefin element to approximately the temperature within said mixture application enclosure;

angling at least some of said plurality of nozzles in a direction of travel of said conveyor;

running said thermoplastic polyolefin element through said mixture application enclosure on said conveyor while said mixture is emitted by said plurality of nozzles, thereby causing said mixture to flow over said thermoplastic polyolefin element;

regulating, during application of said mixture to said thermoplastic polyolefin element, one or more of a flow rate of said mixture, a discharge pattern of said plurality of nozzles, a distance of said plurality of nozzles from said thermoplastic polyolefin element, the orientation of said thermoplastic polyolefin element on said conveyor, and the speed of said conveyor; and

passing said thermoplastic polyolefin element through a drying enclosure after application of said mixture;

whereby a dried layer of said adhesion promoter is thereafter retained on the surface of said thermoplastic polyolefin element; and

## 13

wherein application of said mixture to said thermoplastic polyolefin element in such a manner results in a reduction in the amount of foaming and splashing of said mixture, thereby reducing or eliminating defects in said dried layer of adhesion promoter, which defects would otherwise be inherently visible in said paint coat.

74. The method of claim 73, wherein the average flow rate of said mixture through said plurality of nozzles is between about 0.5–2.5 liters per minute.

75. The method of claim 73, wherein the distance between said plurality of nozzles and the surface of said thermoplastic polyolefin element is between about 0.25–14 inches.

76. The method of claim 73, wherein there are between about 15–30 total nozzles.

77. The method of claim 73, wherein the diameter of said plurality of nozzles is between approximately 0.25–0.5 inches.

78. The method of claim 73, wherein the opening diameter of said plurality of nozzles is between approximately 0.5–1.0 millimeters.

79. The method of claim 73, wherein said at least some of said plurality of nozzles are oriented at an angle of between about 10–45 degrees relative to vertical.

80. The method of claim 73, wherein the linear velocity of said thermoplastic polyolefin element on said conveyor is between about 1–5 meters per minute.

81. The method of claim 73, wherein said thermoplastic polyolefin element is angled toward a direction of travel of said conveyor.

82. The method of claim 81, wherein said angle is between about 5–20 degrees.

83. The method of claim 73, further comprising cleaning said thermoplastic polyolefin element prior to said application of said mixture.

84. The method of claim 83, further comprising rinsing said thermoplastic polyolefin element with de-ionized water prior to application of said mixture.

85. The method of claim 73, wherein said thermoplastic polyolefin element is cooled to a temperature of between about 20–25° C.

## 14

86. The method of claim 73, wherein said atmosphere within said mixture application enclosure is maintained at between approximately 40–70% relative humidity.

87. The method of claim 73, wherein the amount of adhesion promoter mixed with water is regulated by a metering device.

88. The method of claim 87, wherein a surface tension meter is adapted to analyze a wet sample of said mixture, said surface tension meter communicating with said metering device to provide regulation of the amount of said adhesion promoter added to said water based on said analysis.

89. The method of claim 73, wherein said water is de-ionized water.

90. The method of claim 73, further comprising re-circulating said mixture within said mixture storage tank.

91. The method of claim 90, further comprising filtering said mixture during re-circulation.

92. The method of claim 73, further comprising passing said mixture through a heat exchanger to regulate the temperature of said mixture prior to application by said plurality of nozzles.

93. The method of claim 92, wherein a pump supplies said mixture from said heat exchanger to said gravity tank.

94. The method of claim 73, further comprising the use of an air seal for sealing each end of said mixture application enclosure.

95. The method of claim 94, wherein said air seal is provided by a fan.

96. The method of claim 73, wherein the temperature within said drying enclosure is between about 45–95° C.

97. The method of claim 73, wherein the relative humidity within said drying enclosure is between about 5–25%.

98. The method of claim 73, further comprising passing said thermoplastic polyolefin element through a pre-oven prior to its introduction to said drying enclosure.

99. The method of claim 98, wherein the temperature within said pre-oven is between about 25–65° C.

100. The method of claim 98, wherein the relative humidity within said pre-oven is between about 15–60%.

\* \* \* \* \*